

# United States Patent Office

2,911,312  
Patented Nov. 3, 1959

1

2,911,312

## NON-TOXIC ALUMINUM ENAMEL FRITS

Lewis C. Hoffman, Scotch Plains, N.J., assignor to E. I. du Pont de Nemours and Company, Wilmington, Del., a corporation of Delaware

No Drawing. Application January 7, 1957  
Serial No. 632,662

6 Claims. (Cl. 106—48)

This invention relates to new non-toxic aluminum 15 enamel frits. More particularly, it relates to the formation on aluminum and aluminum alloy articles of hard vitreous enamel coatings which will be non-toxic in use, and to certain improved novel vitreous enamel frits to be utilized for such purpose.

Vitreous enamel frits suitable for use in the vitreous enameling of aluminum and aluminum alloy surfaces are described and claimed in Deyrup U.S. Letters Patent No. 2,467,114. Such enamel frits have come into worldwide usage with great success. These Deyrup enamels have even been used for enameling outer surfaces of aluminum cooking utensils. They have not been approved for the enameling of the interior surfaces of such utensils because of possible toxicity when contacted for prolonged periods with certain acidic foodstuffs. It has been theorized that the presence of the substantial lead content of the Deyrup enamels might lead to toxicity to very sensitive persons when acidic foodstuffs are left to stand in such vessels.

Attempts made heretofore to produce a satisfactory vitreous enamel frit for the enameling of aluminum and aluminum alloys without the use of a substantial quantity of lead have been unsuccessful. A satisfactory enamel frit for this purpose should have a melting point less than about 550° C., must be glossy and have good adherence to aluminum, and must have a temperature coefficient of expansion approaching that of aluminum and aluminum alloys.

It is an object of this invention to produce a substantially lead-less, non-toxic vitreous enamel frit satisfactory for enameling aluminum and aluminum alloys.

It is another object of this invention to provide a satisfactory method of enameling aluminum and aluminum alloys with such lead-less, non-toxic enamel frit.

Other objects of this invention will appear hereinafter.

The objects of this invention may be accomplished by the preparation of a non-toxic, substantially lead-less

2

enamel frit having a maturing temperature of 490° C.—550° C., at least 70% by weight of said frit consisting of

22-35% by weight  $TiO_2$   
14-29% by weight  $SiO_2$   
17-26% by weight  $Na_2O$   
1-3% by weight  $Li_2O$   
said frit containing less than  
4.0% by weight  $Al_2O_3$   
11.0% by weight  $B_2O_3$   
30.0% by weight  $BaO$   
4.0% by weight  $CaO$   
1.0% by weight  $CoO$   
0.5% by weight  $CdO$   
11.0% by weight  $K_2O$   
0.1% by weight  $MnO$   
0.1% by weight  $NiO$   
0.5% by weight  $PbO$   
2.0% by weight  $ZnO$   
4.0% by weight  $ZrO_2$

20 All percentages of ingredients are expressed in weight percent for convenience of comparison with prior art.

Although the enamel frits above characterized are entirely suitable for the formation of protective, adherent and attractive enamel coatings on aluminum and aluminum alloys, there is sometimes evidence of corrosion of the aluminum surface during the firing operation. Such corrosion appears to be the result of firing of the particular enamel composition of this invention since it does not appear in the firing of the Deyrup enamels which contain

25 substantial quantities of lead oxide. I have now discovered that this corrosion during firing, evidenced by slight unevenness of coated surface, can be eliminated by addition to the frit composition, before melting, of 1% to 11%  $Sb_2O_3$ . It is, therefore, generally preferred that such quantity of antimony oxide be molten in the frit composition. Preferably, the amount of  $Sb_2O_3$  melted in the frit composition will be between 1% and 5%. The amount required will depend upon the alkali content of the frit, the amount of chromate pretreatment that the aluminum surface is subjected to, and whether the surface is substantially pure aluminum or the aluminum content is an aluminum alloy. The lower the alkali content of the frit, the lower may the  $Sb_2O_3$  content be to obtain a given effect. Tables 1 and 2, below, show preferred exemplary enamel frit compositions in weight percent and mol percent, respectively. Table 3 discloses weight percent composition of batches for the production of the respective enamel frits shown in Tables 1 and 2.

30 35 40 45 50 It is to be understood that other suitable batch compositions may be used in making the respective frits of Tables 1 and 2, the raw materials being calculated to yield the desired frit composition.

TABLE I

[Weight percent]

|                |       |       |       |       |       |       |       |       |       |       |       |       |       |       |
|----------------|-------|-------|-------|-------|-------|-------|-------|-------|-------|-------|-------|-------|-------|-------|
| $Li_2O$        | 1.6   | 1.7   | 1.6   | 1.6   | 1.9   | 1.9   | 2.1   | 1.5   | 1.6   | 1.4   | 1.8   | 1.8   | 1.8   | 2.0   |
| $Na_2O$        | 20.9  | 22.0  | 20.7  | 20.7  | 21.4  | 21.5  | 21.5  | 19.7  | 21.9  | 17.0  | 23.7  | 20.5  | 24.4  | 25.4  |
| $K_2O$         | 9.7   | 10.2  | 9.6   | 9.6   | 6.0   | 7.3   | ----- | 9.2   | 8.7   | 7.4   | 6.5   | 5.9   | 9.7   | 10.6  |
| Total $R_2O$   | 32.2  | 33.9  | 31.9  | 31.9  | 29.3  | 30.7  | 23.6  | 30.4  | 32.2  | 25.8  | 32.0  | 28.2  | 35.9  | 38.0  |
| $CaO$          | 1.2   | ----- | ----- | ----- | ----- | ----- | ----- | ----- | ----- | ----- | ----- | 3.3   | ----- | ----- |
| $BaO$          | 10.4  | 10.9  | 10.2  | 10.2  | 12.6  | 11.1  | 13.6  | 9.7   | 18.7  | 30.3  | 11.2  | 11.3  | ----- | ----- |
| $ZnO$          | ----- | ----- | ----- | ----- | 2.0   | ----- | ----- | ----- | ----- | ----- | ----- | ----- | ----- | ----- |
| Total $RO$     | 11.6  | 10.9  | 10.2  | 10.2  | 12.6  | 13.1  | 13.6  | 9.7   | 18.7  | 30.3  | 11.2  | 14.6  | ----- | ----- |
| $Al_2O_3$      | ----- | ----- | ----- | ----- | 3.5   | ----- | ----- | ----- | ----- | ----- | ----- | ----- | 3.3   | ----- |
| $B_2O_3$       | 6.5   | 1.7   | 1.6   | 1.6   | 9.7   | 9.7   | 10.5  | 1.5   | ----- | ----- | 1.7   | 1.7   | 7.2   | ----- |
| $Sb_2O_3$      | 1.7   | 1.6   | 1.9   | 1.9   | ----- | 2.1   | 1.5   | ----- | ----- | ----- | 1.7   | 1.7   | 1.8   | 1.8   |
| Total $R_2O_3$ | 6.5   | 3.4   | 3.2   | 6.7   | 11.6  | 9.7   | 12.6  | 3.0   | ----- | ----- | 3.4   | 3.4   | 9.0   | 1.8   |
| $SiO_2$        | 23.4  | 24.4  | 23.0  | 23.1  | 14.6  | 14.6  | 15.8  | 22.0  | 23.2  | 19.9  | 25.2  | 25.4  | 26.0  | 28.4  |
| $TiO_2$        | 26.2  | 27.4  | 23.1  | 23.1  | 31.8  | 31.9  | 34.5  | 34.9  | 26.0  | 22.3  | 28.2  | 28.5  | 29.1  | 31.9  |
| $ZrO_2$        | ----- | 3.6   | ----- | ----- | ----- | ----- | ----- | ----- | ----- | ----- | ----- | ----- | ----- | ----- |
| Total $RO_2$   | 49.6  | 51.8  | 54.7  | 51.2  | 46.4  | 46.5  | 50.3  | 66.9  | 49.2  | 42.2  | 53.4  | 53.9  | 55.1  | 60.2  |

TABLE 2  
[Mol percent]

|                                     |      |      |      |      |      |      |      |      |      |      |      |      |      |      |
|-------------------------------------|------|------|------|------|------|------|------|------|------|------|------|------|------|------|
| Li <sub>2</sub> O                   | 3.8  | 4.2  | 3.9  | 3.9  | 4.7  | 4.6  | 5.2  | 3.7  | 4.0  | 3.9  | 4.3  | 4.3  | 4.1  | 4.6  |
| Na <sub>2</sub> O                   | 24.2 | 25.9 | 24.7 | 24.6 | 25.7 | 25.4 | 25.6 | 23.4 | 26.4 | 22.7 | 27.5 | 23.7 | 26.9 | 27.9 |
| K <sub>2</sub> O                    | 7.4  | 7.9  | 7.6  | 7.5  | 4.8  | 5.7  | 5.7  | 7.2  | 7.0  | 6.5  | 5.0  | 4.5  | 7.0  | 7.7  |
| Total R <sub>2</sub> O              | 35.4 | 38.0 | 36.2 | 36.0 | 35.2 | 35.7 | 30.8 | 34.3 | 37.4 | 33.1 | 36.8 | 32.5 | 38.0 | 40.2 |
| CaO                                 | 1.5  |      |      |      |      |      |      |      |      |      |      | 4.2  |      |      |
| BaO                                 | 4.9  | 5.2  | 5.0  | 5.0  | 6.1  | 5.3  | 6.5  | 4.6  | 9.2  | 16.4 | 5.3  | 5.3  |      |      |
| ZnO                                 |      |      |      |      |      | 1.8  |      |      |      |      |      |      |      |      |
| Total RO                            | 6.4  | 5.2  | 5.0  | 5.0  | 6.1  | 7.1  | 6.5  | 4.6  | 9.2  | 16.4 | 5.3  | 9.5  |      |      |
| Al <sub>2</sub> O <sub>3</sub>      |      |      |      |      |      | 2.5  |      |      |      |      |      |      |      |      |
| B <sub>2</sub> O <sub>3</sub>       | 6.7  | 1.8  | 1.7  | 1.7  | 10.4 | 10.2 | 11.1 | 1.6  |      |      | 1.7  | 1.7  | 7.0  |      |
| Sn <sub>2</sub> O <sub>3</sub>      |      | 0.4  | 0.5  | 0.4  | 0.5  |      | 0.5  | 0.4  |      |      | 0.4  | 0.4  | 0.4  | 0.4  |
| Total R <sub>2</sub> O <sub>3</sub> | 6.7  | 2.2  | 2.2  | 4.6  | 10.9 | 10.2 | 11.6 | 2.0  |      |      | 2.1  | 2.1  | 7.4  | 0.4  |
| SiO <sub>2</sub>                    | 28.0 | 29.7 | 28.4 | 28.4 | 18.1 | 17.8 | 19.4 | 27.0 | 29.0 | 27.4 | 30.3 | 30.3 | 30.0 | 32.2 |
| TiO <sub>2</sub>                    | 23.6 | 25.0 | 26.1 | 25.9 | 29.7 | 29.2 | 31.7 | 32.1 | 24.4 | 23.1 | 25.5 | 25.6 | 24.6 | 27.2 |
| ZrO <sub>2</sub>                    |      |      | 2.2  |      |      |      |      |      |      |      |      |      |      |      |
| Total RO <sub>2</sub>               | 51.6 | 54.7 | 56.7 | 54.3 | 47.8 | 47.0 | 51.1 | 59.1 | 53.4 | 50.5 | 55.8 | 55.9 | 54.6 | 59.4 |

TABLE 3  
[Weight percent]

|                                                                      | 1    | 2    | 3    | 4    | 5    | 6    | 7    | 8    | 9    | 10   | 11   | 12   | 13   | 14   |
|----------------------------------------------------------------------|------|------|------|------|------|------|------|------|------|------|------|------|------|------|
| Flint (SiO <sub>2</sub> )                                            | 17.7 | 19.0 | 16.7 | 18.6 | 10.8 | 10.9 | 11.9 | 17.5 | 18.1 | 15.5 | 19.7 | 19.9 | 19.8 | 21.5 |
| Boric Acid (H <sub>3</sub> BO <sub>3</sub> )                         | 2.2  | 2.3  | 2.2  | 2.3  | 12.8 | 13.0 | 14.2 | 2.1  |      |      | 2.4  | 2.4  | 9.8  |      |
| Titanium Oxide (TiO <sub>2</sub> )                                   | 19.8 | 21.3 | 22.1 | 22.6 | 23.5 | 23.8 | 26.1 | 27.8 | 20.3 | 17.3 | 22.1 | 22.3 | 22.2 | 24.1 |
| Barium Carbonate (BaCO <sub>3</sub> )                                | 10.2 | 10.9 | 10.5 | 10.7 | 12.1 | 10.7 | 13.4 | 10.1 | 18.9 | 30.6 | 11.3 | 11.5 |      |      |
| Whiting (CaCO <sub>3</sub> )                                         | 1.7  |      |      |      |      |      |      |      |      |      |      | 4.7  |      |      |
| Zinc Oxide (ZnO)                                                     |      |      |      |      |      |      | 1.5  |      |      |      |      |      |      |      |
| Antimony Oxide (Sb <sub>2</sub> O <sub>3</sub> )                     |      | 1.3  | 1.2  | 1.3  | 1.4  |      | 1.6  | 1.2  |      |      | 1.3  | 1.4  | 1.4  | 1.5  |
| Aluminum Hydrate (Al <sub>2</sub> O <sub>3</sub> ·3H <sub>2</sub> O) |      |      |      | 4.4  |      |      |      |      |      |      |      |      |      |      |
| Zircon Sand (67% ZrO <sub>2</sub> -33% SiO <sub>2</sub> )            |      |      |      | 4.3  |      |      |      |      |      |      |      |      |      |      |
| Soda Ash (Na <sub>2</sub> CO <sub>3</sub> )                          | 26.0 | 28.0 | 26.7 | 27.3 | 25.9 | 26.3 | 26.5 | 25.7 | 26.6 | 22.7 | 29.0 | 24.6 | 29.0 | 31.6 |
| Potash (K <sub>2</sub> CO <sub>3</sub> )                             | 10.8 | 11.6 | 11.1 | 11.4 | 7.9  | 8.0  |      | 10.7 | 11.1 | 9.5  | 8.4  | 7.5  | 12.8 | 13.2 |
| Lithium Carbonate (Li <sub>2</sub> CO <sub>3</sub> )                 | 3.0  | 3.3  | 3.1  | 3.2  | 3.6  | 3.6  | 4.0  | 3.0  | 3.1  | 2.6  | 3.4  | 3.4  | 3.4  | 5.7  |
| Sodium Nitrate (NaNO <sub>3</sub> )                                  | 2.1  | 2.2  | 2.1  | 2.2  | 2.0  | 2.2  | 2.4  | 2.0  | 2.1  | 1.8  | 2.3  | 2.3  | 2.3  | 2.5  |

In preparing the frits, the batch is weighed, mixed, and heated in a crucible until completely melted to a homogeneous mass. Crucible temperatures may vary from 900° C. to 1200° C. The molten glass is fritted by running the molten mass into water which causes a shattering of the glass into small particles to form the frit. The frit may be dried at about 50° C. or less to remove the water therefrom.

The frit is then customarily ground in a ball mill or other mill in the presence of water or other liquid, or in some cases by dry grinding. During grinding it is convenient to include so-called mill addition agents such as white or colored pigments, opacifying agents, or the like. Suitable dispersing and bonding agents may also be added to the mill.

The dispersion or suspension of the powdered enamel in a suitable vehicle may be applied to the aluminum surface in the customary manner by spraying, dipping, stenciling, brushing, etc. Any air-dry or thermo-fluid vehicle heretofore used in preparing dispersions or suspensions of powdered vitreous enamels may be used for preparation of such dispersions or suspensions of the enamels of this invention. Such vehicles are, for example, disclosed in the following U.S. patents: Deyrup 2,467,114, Andrews 2,682,480, Jessen 2,607,701, and Jessen 2,607,702.

The aluminum or aluminum alloy surfaces to be enameled are first cleaned, if necessary, by treatment with degreasing solvents, or the like. The surfaces should then be pretreated with a chromate solution substantially in the manner described in Deyrup et al. Patent No. 2,544,139. Preferably, the chromate pretreatment of the aluminum surface is slightly more drastic than the particular methods described in Patent No. 2,544,139. For example, the chromate content of the pretreatment bath is preferably above about 10%, expressed as potassium chromate. For example, the following chromate pretreatment has been found very satis-

factory for use in preparing aluminum surfaces for enameling with the enamels of this invention:

NaOH \_\_\_\_\_ grams 330  
K<sub>2</sub>Cr<sub>2</sub>O<sub>7</sub> \_\_\_\_\_ do 667  
Cr<sub>2</sub>(SO<sub>4</sub>)<sub>3</sub> \_\_\_\_\_ do 14.2  
Water \_\_\_\_\_ gallons 1

45 The aluminum article is immersed in this bath, heated to a temperature of 60° C., for a period of two to ten minutes. The pretreated surface is then preferably fired for a period of two to thirty minutes at a temperature between 480° C. and 580° C. The optimum conditions of chromate pretreatment and firing will depend largely upon the composition of the aluminum alloy to be treated.

In the case of any particular aluminum alloy, it can readily be determined whether or not sufficient enamel adherence to insure against water-spalling is obtained by any prescribed course of treatment. This can be determined by means of the following accelerated test which correlates with water exposure results which may take weeks or months. This accelerated test consists in chromate-treating and enameling pieces of the particular alloy to be tested, and then exposing the enamel-metal interface by gouging, filing, or scratching the same, and immersing the test sample in 5% aqueous ammonium chloride solution for ninety-six hours at room temperature.

If no failure occurs back one-eighth inch from the edge of the exposed interface, excellent performance in water exposure will result from the chromate treatment and enameling conditions used. The particular optimum treatment and enameling conditions for a specific alloy can thereby be established. Once optimum treatment conditions for a given alloy have been established and a chromate bath is used for continued treatment of the alloy structures or articles, it will, of course, be desirable to periodically analyze the treating bath and keep the chromate content and alkalinity of the bath within a few percent of their initial value.

After application of the enamel to the aluminum or aluminum alloy, it is fired in a suitable furnace in order to fuse the powdered enamel to a continuous glossy coating. The firing conditions are not critical, except that the article must be brought to a temperature high enough to melt the enamel but not so high that the metal article will be injured. The temperature necessary depends to some extent on the particular aluminum alloy being enameled and upon the particular enamel composition being used. It is not generally necessary to employ a temperature above about 550° C. and, in most cases, the enamel may be satisfactorily fused at a temperature between 490° C. and 550° C. It is merely necessary to keep the article at the selected temperature for a few minutes to permit the enamel to fuse completely to a uniform, adherent, vitreous layer. Several coats may be applied, if desired.

The enamels of this invention have surprisingly low fusion points despite the fact that they do not contain any substantial quantity of lead. Moreover, these enamels have a degree of resistance to chemical agents which was not believed possible for a substantially lead-free enamel. Furthermore, these enamels adhere exceedingly well to aluminum or aluminum alloy surfaces even when exposed to thermal shocks or considerable mechanical flexing of the metal. The following examples are given to illustrate certain preferred procedures for the enameling of aluminum and aluminum alloys.

*Example I*

Aluminum alloy sheet stock composed of aluminum alloy 61 (containing, by weight, 0.25% copper, 0.6% silicon, 1.0% magnesium, and 2.5% chromium) is immersed for two minutes in a bath heated to 60° C. and consisting of the following:

|                                                 |         |      |
|-------------------------------------------------|---------|------|
| NaOH                                            | grams   | 330  |
| K <sub>2</sub> Cr <sub>2</sub> O <sub>7</sub>   | do      | 667  |
| Cr <sub>2</sub> (SO <sub>4</sub> ) <sub>3</sub> | do      | 14.2 |
| Water                                           | gallons | 1    |

After two minutes, the sheet is removed, rinsed in tap water and dried. The sheet is then heat treated at a temperature of about 500° C. for five minutes. The heat-treated sheet after cooling is then dipped into a water slurry of an enamel consisting of

|                                              |
|----------------------------------------------|
| 1.6% by weight Li <sub>2</sub> O             |
| 20.9% by weight Na <sub>2</sub> O            |
| 9.7% by weight K <sub>2</sub> O              |
| 1.2% by weight CaO                           |
| 10.4% by weight BaO                          |
| 6.5% by weight B <sub>2</sub> O <sub>3</sub> |
| 23.4% by weight SiO <sub>2</sub>             |
| 26.2% by weight TiO <sub>2</sub>             |

The liquid and solid contents of the slurry are mixed in such proportions that the sheet after dipping in the slurry and draining will contain approximately 0.5 gram per square inch of surface. The enamel is fired at a temperature of 500° C. for nine minutes. The resulting enamel will have optimum properties; for example, it will be glossy and of a pleasing white color, which will adhere tenaciously to the substrate in life testing and in accelerated testing and it will be substantially unaffected by 10% citric acid in fifteen minutes, and will resist indefinitely the attack of a 10% household detergent solution at boiling temperature.

*Example II*

The process of Example I was repeated using a chromate pretreatment solution containing

|                                                 |         |     |
|-------------------------------------------------|---------|-----|
| NaOH                                            | grams   | 250 |
| K <sub>2</sub> Cr <sub>2</sub> O <sub>7</sub>   | do      | 600 |
| Cr <sub>2</sub> (SO <sub>4</sub> ) <sub>3</sub> | do      | 15  |
| Water                                           | gallons | 1   |

and the use of a frit having the following composition:

|    |                                               |
|----|-----------------------------------------------|
| 5  | 1.7% by weight Li <sub>2</sub> O              |
|    | 22.0% by weight Na <sub>2</sub> O             |
|    | 10.2% by weight K <sub>2</sub> O              |
|    | 10.9% by weight BaO                           |
|    | 1.7% by weight B <sub>2</sub> O <sub>3</sub>  |
|    | 1.7% by weight Sb <sub>2</sub> O <sub>3</sub> |
| 10 | 24.4% by weight SiO <sub>2</sub>              |
|    | 27.4% by weight TiO <sub>2</sub>              |

The other conditions of Example I were followed as set forth in that example. The results were approximately identical to the results therein set forth.

Throughout the specification and claims, any reference to parts, proportions and percentages refers to parts, proportions and percentages by weight unless otherwise specified.

Since many changes and modifications can be made in the above described details without departing from the nature and spirit thereof, it is to be understood that this invention is not to be limited except as set forth in the appended claims.

I claim:

1. A non-toxic vitreous enamel frit having a maturing temperature of 490° C. to 550° C. suitable for the enameling of aluminum and aluminum alloys at least 70% of which consists of

|    |                                        |
|----|----------------------------------------|
| 30 | 22% to 35% TiO <sub>2</sub> by weight  |
|    | 14% to 29% SiO <sub>2</sub> by weight  |
|    | 17% to 26% Na <sub>2</sub> O by weight |
|    | 1% to 3% Li <sub>2</sub> O by weight   |

said frit containing less than

|    |                                               |
|----|-----------------------------------------------|
| 35 | 0.1% NiO by weight                            |
|    | 0.1% MnO by weight                            |
|    | 1.0% CoO by weight                            |
|    | 4.0% Al <sub>2</sub> O <sub>3</sub> by weight |
|    | 11.0% B <sub>2</sub> O <sub>3</sub> by weight |
| 40 | 2.0% ZnO by weight                            |
|    | 30.0% BaO by weight                           |
|    | 4.0% CaO by weight                            |
|    | 4.0% ZrO <sub>2</sub> by weight               |
|    | 0.5% PbO by weight                            |
|    | 11.0% K <sub>2</sub> O by weight              |

45 said frit consisting essentially of the above-named ingredients, all of which are melted together to form the frit.

2. A non-toxic vitreous enamel frit having a maturing temperature of 490° C. to 550° C. suitable for the enameling of aluminum and aluminum alloys at least 70% of which consists of

|    |                                        |
|----|----------------------------------------|
| 55 | 22% to 35% TiO <sub>2</sub> by weight  |
|    | 14% to 29% SiO <sub>2</sub> by weight  |
|    | 17% to 26% Na <sub>2</sub> O by weight |
|    | 1% to 3% Li <sub>2</sub> O by weight   |

said frit containing less than

|    |                                               |
|----|-----------------------------------------------|
| 60 | 0.1% NiO by weight                            |
|    | 0.1% MnO by weight                            |
|    | 1.0% CoO by weight                            |
|    | 4.0% Al <sub>2</sub> O <sub>3</sub> by weight |
|    | 11.0% B <sub>2</sub> O <sub>3</sub> by weight |
|    | 2.0% ZnO by weight                            |
| 65 | 30.0% BaO by weight                           |
|    | 4.0% CaO by weight                            |
|    | 4.0% ZrO <sub>2</sub> by weight               |
|    | 0.5% PbO by weight                            |
|    | 11.0% K <sub>2</sub> O by weight              |

70 said frit consisting essentially of the above-named ingredients, and as an agent to prevent corrosion during firing of the enamel between 1% and 11% Sb<sub>2</sub>O<sub>3</sub>, all of said ingredients being melted together to form said frit.

3. A process for applying a protective coating on the

surface of aluminum and aluminum rich alloys which comprises fusing thereon a vitreous enamel frit having a maturing temperature of 490° C. to 550° C. at least 70% of said enamel frit consisting of

22% to 35%  $TiO_2$  by weight  
14% to 29%  $SiO_2$  by weight  
17% to 26%  $Na_2O$  by weight  
1% to 3%  $Li_2O$  by weight

said frit containing less than

0.1%  $NiO$  by weight  
0.1%  $MnO$  by weight  
1.0%  $CoO$  by weight  
4.0%  $Al_2O_3$  by weight  
11.0%  $B_2O_3$  by weight  
2.0%  $ZnO$  by weight  
30.0%  $BaO$  by weight  
4.0%  $CaO$  by weight  
4.0%  $ZrO_2$  by weight  
0.5%  $PbO$  by weight  
11.0%  $K_2O$  by weight

said frit consisting essentially of the above-named ingredients, all of which are melted together to form the frit.

4. A process for applying a protective coating on the surface of aluminum and aluminum rich alloys which comprises fusing thereon a vitreous enamel frit having a maturing temperature of 490° C. to 550° C. at least 70% of said enamel frit consisting of

22% to 35%  $TiO_2$  by weight  
14% to 29%  $SiO_2$  by weight  
17% to 26%  $Na_2O$  by weight  
1% to 3%  $Li_2O$  by weight

said frit containing less than

0.1%  $NiO$  by weight  
0.1%  $MnO$  by weight  
1.0%  $CoO$  by weight  
4.0%  $Al_2O_3$  by weight  
11.0%  $B_2O_3$  by weight  
2.0%  $ZnO$  by weight  
30.0%  $BaO$  by weight  
4.0%  $CaO$  by weight  
4.0%  $ZrO_2$  by weight  
0.5%  $PbO$  by weight  
11.0%  $K_2O$  by weight

said frit and consisting essentially of the above-named ingredients, and as an agent to prevent corrosion during firing of the enamel between 1% and 11%  $Sb_2O_3$ , all of said ingredients being melted together to form said frit.

5. Aluminum and aluminum rich alloy articles containing a protective coating comprising a non-toxic vitreous

enamel having a maturing temperature of 490° C. to 550° C. at least 70% of said enamel consisting of

22% to 35%  $TiO_2$  by weight  
14% to 29%  $SiO_2$  by weight  
17% to 26%  $Na_2O$  by weight  
1% to 3%  $Li_2O$  by weight

said enamel containing less than

0.1%  $NiO$  by weight  
0.1%  $MnO$  by weight  
1.0%  $CoO$  by weight  
4.0%  $Al_2O_3$  by weight  
11.0%  $B_2O_3$  by weight  
2.0%  $ZnO$  by weight  
30.0%  $BaO$  by weight  
4.0%  $CaO$  by weight  
4.0%  $ZrO_2$  by weight  
0.5%  $PbO$  by weight  
11.0%  $K_2O$  by weight

20 said enamel consisting essentially of the above-named ingredients, all of which are melted together to form the frit of the enamel.

6. Aluminum and aluminum rich alloy articles containing a protective coating comprising a non-toxic vitreous enamel having a maturing temperature of 490° C. to 550° C. at least 70% of said enamel consisting of

22% to 35%  $TiO_2$  by weight  
14% to 29%  $SiO_2$  by weight  
17% to 26%  $Na_2O$  by weight  
1% to 3%  $Li_2O$  by weight

said enamel containing less than

0.1%  $NiO$  by weight  
0.1%  $MnO$  by weight  
1.0%  $CoO$  by weight  
4.0%  $Al_2O_3$  by weight  
11.0%  $B_2O_3$  by weight  
2.0%  $ZnO$  by weight  
30.0%  $BaO$  by weight  
4.0%  $CaO$  by weight  
4.0%  $ZrO_2$  by weight  
0.5%  $PbO$  by weight  
11.0%  $K_2O$  by weight

45 said enamel consisting essentially of the above-named ingredients, and as an agent to prevent corrosion during firing of the enamel between 1% and 11%  $Sb_2O_3$ , all of which said ingredients being melted together to form the enamel frit.

50 References Cited in the file of this patent

#### UNITED STATES PATENTS

|           |                  |               |
|-----------|------------------|---------------|
| 2,414,633 | Bryant           | Jan. 21, 1947 |
| 2,660,531 | Fraser et al.    | Nov. 24, 1953 |
| 2,662,020 | Schofield et al. | Dec. 8, 1953  |
| 2,753,271 | Treptow          | July 3, 1956  |

**Notice of Adverse Decision in Interference**

In Interference No. 92,758 involving Patent No. 2,911,812, L. C. Hoffman, NON-TOXIC ALUMINUM ENAMEL FRITS, final judgment adverse to the patentee was rendered May 31, 1966, as to claims 1 and 2.

*[Official Gazette December 13, 1966.]*

### **Disclaimer**

2,911,312.—*Lewis C. Hoffman*, Scotch Plains, N.J. NON-TOXIC ALUMINUM ENAMEL FRITS. Patent dated Nov. 3, 1959. Disclaimer filed Aug. 12, 1966, by the inventor and the assignee, *E. I. du Pont de Nemours and Company*.

Hereby enters this disclaimer as to claims 1 and 2 of said patent.  
[*Official Gazette December 20, 1966.*]